

## UNITED STATES PATENT OFFICE

2,610,128

## SILK-SCREEN PRINTING PASTE

Frank Enoch Kerridge and Cyril Stanley Couper,  
London, England, assignors to Johnson, Mat-  
they & Company Limited, London, England, a  
British company

No Drawing. Application July 18, 1949, Serial No.  
105,444. In Great Britain July 27, 1948

5 Claims. (Cl. 106—26)

1

This invention relates to improvements in and relating to the decoration of heat-resisting bases, that is to say bases capable of withstanding firing at a temperature of at least 400° C., such as glass, earthenware and china and is more particularly concerned with the decoration of such bases with a design or decoration in platinum, or having a platinum or silver-like appearance.

Platinum decorations, or decorations having a platinum or silver appearance have in general heretofore been produced on glass, china or earthenware by the use of one of the following materials, namely:

(1) "Liquid platinum" which consists essentially of a solution of platinum sulphoresinate in suitable solvents;

(2) "Liquid white gold" (popularly known as "liquid silver") which consists essentially of a mixture, in suitable solvents, of platinum and gold sulphoresinates, a mixture of palladium and gold sulphoresinates, or a mixture of platinum, palladium, and gold sulphoresinates;

(3) "Liquid burnish white gold" (sometimes known as "liquid burnish silver") consisting of a suspension of gold or a gold compound in a solution of gold and platinum sulphoresinates, or of gold and palladium sulphoresinates, and, in some cases, including a mercury compound;

(4) Finely divided (usually precipitated) platinum powder, with or without a powdered mercury compound;

(5) Finely divided platinum or palladium, with gold powder, with or without a powdered mercury compound.

All of the above materials contain an adhesion-promoting agent, which, in the case of those materials consisting only of sulphoresinate solutions, is usually bismuth resinate and, in the case of those containing powder or a powder suspension, is a lead borosilicate flux or bismuth oxide or oxychloride.

In the decoration of articles with a single simple design in platinum, or having a platinum or silver-like appearance, each of the above may be applied by hand painting with subsequent firing. When, however, a repetitive design is required to be applied to the ware, it is usual to apply the decoration by a printing method, namely rubber stamp printing or engraved plate printing.

The rubber stamp method, whilst being simple and rapid in use, results in a design which is lacking in richness and sharpness of outline and, moreover, does not enable ceramic colours to be

2

printed simultaneously in register with the platinum, or platinum-like decoration.

With engraved plate or copper plate printing a transfer is prepared by engraving or etching a design on a copper or glass plate, filling the interstices or depressions so formed with the printing paste, applying a sheet of gummed tissue paper, gummed side downwards to the coated plate and then removing the paper, which now carries the design. To decorate an article, the paper is applied, whilst the paste is still moist or sticky with the design-carrying side downwards, to the article. The tissue paper is then soaked off and the article fired.

This method, in the hands of a skilled operator, gives a decoration of good quality, but, as the design is applied to the ware in the moist state, it cannot be used for applying both platinum, or a platinum-like decoration and a ceramic colour simultaneously in register. A further disadvantage is that transfers prepared by this method cannot normally be stored for future use. It is also known to decorate ware with a ceramic colour or vitreous enamel by applying directly to the ware a vitreous enamel or ceramic colour paste by means of the silk-screen printing method and it has also been proposed to prepare a ceramic colour transfer by the silk-screen printing method.

Silk-screen printing, whether used for decorating an article by direct application or for the preparation of transfers, offers advantages over the other methods referred to in that the apparatus employed is inexpensive, a variety of decorative effects are obtainable and prints of high quality and well-defined outlines can be readily produced by relatively unskilled workers.

Pastes embodying the above mentioned materials as heretofore constituted for use with the rubber stamp or engraved plate printing methods are quite unsuited for use with the silk-screen printing method, particularly in the case of the preparation of transfers.

It will be appreciated from a consideration of the above that, if a platinum paste or one giving a platinum or silver-like appearance, were provided, which could be satisfactorily applied by the silk-screen printing method, very considerable advantages would accrue both from the artistic and the commercial aspects. In the first place, it would be possible to decorate an article with a design in platinum, which would have a more pleasing effect than those hitherto obtainable with the hitherto known methods, owing to the improved definition of the outlines and the fact

that it becomes possible to print a ceramic colour design in register with the platinum, and secondly, the process of decorating can be carried out relatively inexpensively.

Silk-screen printing, however, produces a very thick deposit and whilst this is in many instances, particularly in the case of ceramic enamels, greatly to be desired, it may be that, in the case of a platinum decoration, the cost of the platinum may outweigh the advantages attainable by the use of his method. Attempts to produce a thinner deposit by employing a low platinum, or like precious metal, to medium ratio will result in unsatisfactory printing owing to the low proportion of solid in the paste, and frequently in flowing of the prints and loss of sharpness of outline before drying.

An object of the invention is to overcome the above disadvantages and to provide an improved platinum paste suitable for direct application to an article to be decorated by the silk-screen printing method or for the preparation by the silk-screen printing method, of transfers intended for subsequent application to an article.

Another object is to enable a thin deposit of platinum to be applied to a heat resisting base by the silk-screen printing method.

A further object is to enable the thickness of the platinum deposit to be readily controllable.

Another object is to provide a silk-screen printing paste including platinum powder and a volatilisable solid, which will volatilise without carbonising during the subsequent firing of a heat-resisting base decorated with the paste.

A still further object is to provide a silk-screen printing paste comprising platinum powder, a flux or adhesion promoting agent having a melting point not higher than 500° C., an organic silk-screen printing medium or vehicle, and a volatilisable solid.

By including a volatilisable solid in the paste, the amount of precious metal in the paste, and hence the thickness of the final precious metal film obtained after firing, may be varied as desired, since by suitably proportioning the amount of volatilisable solid included, the ratio of liquid to total solids in the paste may be maintained in the correct proportion to give good printing qualities.

The volatilisable solid may consist of any solid which volatilises completely at a low temperature, but we have found that certain organic materials, such as oxanilide, acetanilide or anthracene are more suitable than volatilisable inorganic materials, such as ammonium chloride. Of the organic materials mentioned, we prefer to use anthracene.

The proportion of medium to solid substances is preferably 1-4 parts of medium to 2 parts of solid, the exact proportions depending on the particle size of the solids and the viscosity of the medium.

The organic medium will comprise a film-forming ingredient dissolved in a solvent, for example it may be a cellulose derivative or a natural or synthetic resin or resins or a mixture thereof dissolved in a solvent or solvent mixture having a rate of evaporation suitable for silk-screen printing. For example, the medium may consist of nitrocellulose dissolved in amyl and/or ethyl lactate or of colophony dissolved in pine oil.

The flux may be a lead borosilicate or a lead alkali borosilicate flux or a bismuth compound, such as bismuth oxide or oxychloride.

If desired, an extender such as a mercury salt, may be included in the paste. In this case, we prefer to use mercurous chloride.

If the paste is to be used to prepare a transfer, it will be found desirable to include in the medium a suitable plasticiser or plasticisers, such as methyl abietate and/or castor oil for the purpose of preventing cracking of the decoration during firing.

The following are examples of pastes prepared in accordance with the invention for the decoration of glass, containing a cellulose derivative-based and a resinous medium respectively:

|                                   | Per cent by weight |
|-----------------------------------|--------------------|
| (1) Platinum powder               | 40                 |
| Mercurous chloride                | 10                 |
| Low fusing lead borosilicate flux | 3.5                |
| Volatilisable solid (anthracene)  | 2.5                |
| Plasticised nitrocellulose medium | 44                 |

the constituents being ground together to form a paste.

|                                   | Per cent by weight |
|-----------------------------------|--------------------|
| (2) Platinum powder               | 40                 |
| Mercurous chloride                | 10                 |
| Low fusing lead borosilicate flux | 3.5                |
| Volatilisable solid (anthracene)  | 2.5                |
| Plasticised resinous medium       | 44                 |

the constituents being ground together to form a paste.

In the case of the decoration of a pottery article, a lower percentage of flux may be used, since a higher firing temperature can be employed than with glass.

The preferred composition of the individual constituents of our improved paste is as follows:

|    | Flux or adhesion promoting constituent                                                                                                                                                                                                                            |
|----|-------------------------------------------------------------------------------------------------------------------------------------------------------------------------------------------------------------------------------------------------------------------|
| 40 | Although many lead borosilicate or lead alkali borosilicate fluxes which melt at a temperature of 400-500° C., or a bismuth compound may be used, we have found that the most satisfactory results are obtained by using a flux having the following composition: |
| 45 | Lead monoxide (PbO) 85.5                                                                                                                                                                                                                                          |
|    | Boric oxide (B <sub>2</sub> O <sub>3</sub> ) 7.0                                                                                                                                                                                                                  |
|    | Silica (SiO <sub>2</sub> ) 7.5                                                                                                                                                                                                                                    |

|    | Per cent by weight                               |
|----|--------------------------------------------------|
| 50 | Lead monoxide (PbO) 85.5                         |
|    | Boric oxide (B <sub>2</sub> O <sub>3</sub> ) 7.0 |
|    | Silica (SiO <sub>2</sub> ) 7.5                   |

|    | Medium                                                                                                     |
|----|------------------------------------------------------------------------------------------------------------|
| 55 | If a medium based on a cellulose derivative is employed, the following composition will be found suitable: |
| 60 | Per cent by weight                                                                                         |
|    | Amyl lactate 56                                                                                            |
|    | Ethyl lactate 20                                                                                           |
|    | Nitrocellulose (medium viscosity) 8                                                                        |
|    | Methyl abietate 8                                                                                          |
|    | Castor oil 8                                                                                               |

If a resinous medium is employed, the following composition will be found suitable:

|    | Per cent by weight |
|----|--------------------|
| 65 | Pine oil 70        |
|    | Colophony 20       |
|    | Methyl abietate 5  |
|    | Castor oil 5       |

In the use of our improved paste for the decoration, for example, of a substantially flat article of glass, the paste is applied to the article, so as to form any desired design thereon, by the silk-screen printing method, and allowed to dry. The coated article is then fired at a temperature

within the range of 500-650° C. depending on the type of glass, to burn away the organic matter and cause the precious metal or metals to adhere firmly to the article.

If the base being decorated is of earthenware or china, the firing temperature is preferably between 650° and 800° C.

The decoration, after firing, will present a matt surface, and should be lightly scoured with sand or burnished with agate so as to produce a bright effect.

When the paste is to be used for preparing a transfer, the paste is applied, in any desired design, to a sheet of transfer paper by the silk-screen printing method and is again allowed to dry. To decorate an article, the transfer paper with the design thereon is applied to the article and the design transferred to the surface thereof by the well-known "slide-off" method. The article is then fired at a suitable temperature, i. e. within the range of 500-650° C. in the case of a glass article and 650-800° C. in the case of earthenware or china. The fired design may, in this case also, be lightly burnished. It is to be understood that the improved paste may be printed so as to register with a vitreous enamel or ceramic colour in a combined platinum or silver-like and enamel decoration.

As will be appreciated, our invention enables an article to be provided with a decoration having the appearance of silver, but which does not tarnish on exposure to air.

What we claim is:

1. A silk-screen printing paste for the preparation of a transfer or for direct application to a heat-resisting base, said paste comprising a mixture of platinum powder, anthracene, a ceramic flux and an organic vehicle consisting of 56% by weight of amyl lactate, 20% by weight of ethyl lactate, 8% by weight of nitrocellulose, 8% by weight of methyl abietate and 8% by weight of castor oil and the relative proportions of platinum powder, ceramic flux and anthracene to liquid vehicle being always substantially 2 parts of solids to 1-4 parts of vehicle.

2. A silk-screen printing paste for the preparation of a transfer or for direct application to a glass base, said paste comprising a mixture of the following constituents in the following proportions by weight, namely:

|                                                | Per cent |
|------------------------------------------------|----------|
| Platinum powder                                | 40       |
| Mercurous chloride                             | 10       |
| Lead borosilicate flux                         | 3.5      |
| Anthracene                                     | 2.5      |
| Solution containing plasticized nitrocellulose | 44       |

3. A silk-screen printing paste for the preparation of a transfer or for direct application to a heat-resisting base, said paste consisting essentially of a platinum powder-ceramic flux mixture and anthracene, said platinum powder-ceramic flux and anthracene constituting solid ingredients, and an organic screening vehicle comprising

ing nitrocellulose dissolved in a solvent selected from the group consisting of amyl lactate, ethyl lactate and mixtures thereof, and the relative proportion of the combined amounts of platinum powder-ceramic flux mixture and anthracene to liquid vehicle being always substantially two parts of solids to 1-4 parts of vehicle.

4. A silk-screen printing paste for the preparation of a transfer or for direct application to a heat-resisting base, said paste consisting essentially of a platinum powder-lead borosilicate flux mixture and anthracene, said platinum powder-lead borosilicate flux and anthracene constituting solid ingredients, and an organic screening vehicle comprising nitrocellulose dissolved in a solvent selected from the group consisting of amyl lactate, ethyl lactate and mixtures thereof, and the relative proportion of the combined amounts of platinum powder-lead borosilicate flux mixture and anthracene to liquid vehicle being always substantially 2 parts of solids to 1-4 parts of vehicle.

5. A silk-screen printing paste for the preparation of a transfer or for direct application to a heat-resisting base, said paste consisting essentially of a platinum powder-ceramic flux mixture, said ceramic flux being selected from the group consisting of bismuth oxide and bismuth oxychloride, and anthracene, said platinum powder-ceramic flux and anthracene constituting solid ingredients, and an organic screening vehicle comprising nitrocellulose dissolved in a solvent selected from the group consisting of amyl lactate, ethyl lactate and mixtures thereof, and the relative proportion of the combined amounts of platinum powder-ceramic flux mixture and anthracene to liquid vehicle being always substantially 2 parts of solids to 1-4 parts of vehicle.

FRANK ENOCH KERRIDGE.  
CYRIL STANLEY COUPER.

#### REFERENCES CITED

The following references are of record in the file of this patent:

| UNITED STATES PATENTS |                  |                |
|-----------------------|------------------|----------------|
| Number                | Name             | Date           |
| 255,421               | Dode             | Mar. 28, 1882  |
| 460,358               | Buttler          | Sept. 29, 1891 |
| 1,752,462             | Smith            | Apr. 1, 1930   |
| 2,113,449             | Hoffman et al.   | Apr. 5, 1938   |
| 2,190,210             | Kaber            | Feb. 13, 1940  |
| 2,287,053             | Murphy           | June 23, 1942  |
| 2,294,760             | Morris           | Sept. 1, 1942  |
| 2,318,803             | Schneider et al. | May 11, 1943   |
| 2,452,805             | Sussenbach       | Nov. 2, 1948   |

#### FOREIGN PATENTS

|         | Country       | Date           |
|---------|---------------|----------------|
| 7,688   | Great Britain | 1892           |
| 9,261   | Great Britain | 1894           |
| 428,743 | Great Britain | May 17, 1935   |
| 526,853 | Great Britain | Sept. 26, 1940 |
| 566,718 | Great Britain | June 10, 1945  |